

## UNITED STATES PATENT OFFICE.

JAMES HENRY REID, OF READSBORO, VERMONT, ASSIGNOR TO INTERNATIONAL NITROGEN COMPANY, OF CLEVELAND, OHIO, A CORPORATION OF DELAWARE.

PROCESS OF AND MATERIAL FOR THE PRODUCTION OF CARBIDE AND REDUCTION OF ORE.

No Drawing.

Application filed January 27, 1921. Serial No. 440,342.

To all whom it may concern:

Be it known that I, JAMES HENRY REID, a citizen of the United States, residing at Readsboro, in the county of Bennington and State of Vermont, have invented a certain new and useful Improvement in Processes of and Material for the Production of Carbide and Reduction of Ore, of which the following is a full, clear, and exact description.

This invention relates to a process of and material for the production of carbide and reduction of ore. The general object of the invention is to provide a process whereby the production of the carbide and the reduction of the ore may be accomplished simultaneously and efficiently and, in connection with such production and reduction, to generate a large quantity of gas of a heating value useful in the industrial arts. Further objects and advantages of the invention will appear hereinafter in connection with the detailed description of the process, which will be explained in connection with the production of calcium carbide and the reduction of iron ore. For the reducing agent, I employ carbon, obtaining the same from bituminous coal. I also employ calcium carbonate (preferably in the commercial form of limestone) as a fluxing agent and as the source of the metal constituent of the carbide. Sufficient coal will be employed to provide the coke necessary for the carbide reaction and for the reduction of the ore, and sufficient limestone will be employed to furnish the metal constituent of the carbide and the fluxing agent for the ore. A mixture for this purpose will consist of the following ingredients in about the following proportions by weight:

Per cent.

|                         |      |
|-------------------------|------|
| Bituminous coal         | 39   |
| Limestone               | 36.1 |
| Iron ore (ferric oxide) | 24.9 |

The limestone will be ground, preferably to a fineness of about forty mesh and the coal to a fineness of about eight mesh, while the ore as generally obtained will ordinarily

be sufficiently fine, with the exception of the nodules, which should also be ground or otherwise broken up. The limestone, coal and ore are then intimately mixed and are retorted for a length of time and at a temperature sufficient to convert the coal into coke. The temperature may vary from 1400 F. to 2600 or 2800 F., and the time required for the operation will vary inversely with the temperature.

By the retorting operation, the coal will have been converted into coke, with the evolution, not only of the gases ordinarily secured by the distillation thereof, but of additional gases produced by the breaking up of the tarry constituents of the coal and through their contact with the glowing particles of limestone and ore. Because of the fact that the retorting operation is conducted in a reducing atmosphere, at least as long as hydrocarbon vapors are present, the limestone will not be converted into lime.

During the coking operation, the charge of ore, coal, and limestone, will have been converted into the following constituents, the ore having been partly reduced during such operation:

|                        | Per cent. |
|------------------------|-----------|
| Iron and ferrous oxide | 24.9      |
| Coke                   | 29.0      |
| Limestone              | 36.1      |
| Gas                    | 10.0      |

The composition of the solid residue from the retorts will be

|                        | Per cent. |
|------------------------|-----------|
| Iron and ferrous oxide | 27.7      |
| Coke                   | 32.2      |
| Limestone              | 40.1      |

and the ingredients will have been formed into a coked mass, the constituent particles of which are firmly knitted together, making a limestone-metal-ore-coke of great strength and one wherein the ingredients are in ideal juxtaposition for subsequent treatment in an electric furnace. Each particle of ore has immediately adjacent thereto the lime-

stone and coke necessary for its reduction, and each particle of limestone has immediately adjacent thereto one or more particles of coke for the carbide reaction.

5 The coked mass from the retort is broken to suitable size and is then charged into an electric carbide furnace, which may be of any type from which the molten material may be withdrawn from time to time. In 10 the furnace, the material is subjected to the action of electricity in the ordinary manner, resulting in the fusing and reduction of the ore and in the production of carbide, the iron and carbide being produced from a common homogeneous charge and through the same operation of the furnace. Owing to the fact that the calcium is in the form of limestone, the carbide reaction will occur at a temperature below 15 that at which the iron will volatilize. During the operation of the furnace, a large quantity of gas (principally carbon monoxide) will be evolved, and this gas may be collected, together with the gases from 20 the retorts, and used for various purposes, such as heating the retorts, running the electric generator which operates the furnace, or for any commercial or industrial purpose.

25 30 Fusion in the electric furnace will produce from 100 lbs. of the solid residue from the retorts the following:

|                   | Lbs. |
|-------------------|------|
| 35 Iron -----     | 12.5 |
| 73% carbide ----- | 25.2 |
| Slag -----        | 28.3 |
| Gas -----         | 24.0 |

But, as the carbide and the slag are mixed, 10 the molten educt from the electric furnace from such 100 lb. charge will be:

|                   | Lbs. |
|-------------------|------|
| Iron -----        | 12.5 |
| 34% carbide ----- | 53.5 |

45 As the molten material accumulates in the furnace it may be withdrawn from time to time into a suitable pot or receptacle where the carbide, owing to its higher point of fusion, will solidify and float upon the molten iron and from which it and the slag can be removed by skimming; or the mixture of carbide and slag may be drawn from the top of the molten iron without waiting 50 for solidification.

55 Although the slag is in excess of the carbide in the mixture therewith, the mixture having the proportion of carbide above set forth is capable of nitrification and of being 60 used direct without dilution of its strength. Furthermore the mixture can be used for the generation of acetylene.

65 By the foregoing process, I have produced, by a single retorting operation, material for the production of carbide and the

reduction of ore; and, by a single treatment in an electric furnace, I have reduced the ore and have produced a grade of carbide that is capable of efficient use, particularly 70 in the production of nitrified material. Furthermore, in the practice of the process, I have been enabled to obtain from a given quantity of cokable coal a quantity of gas not only valuable for use in the industrial arts, but greatly in excess of the quantity 75 which has heretofore been considered as obtainable from the same.

In the process as thus particularly described, I have selected iron as the metal 80 ingredient of the ore and calcium as the metal ingredient of the fluxing agent, for the reason that the said ore is the one most used in the arts and because carbide of calcium is the one generally used for the preparation of nitrified material. However, by 85 using silica in place of the limestone, we have a fluxing agent which is capable of producing silicon carbide, or carborundum; and an impure carborundum (containing 90 slag in the proportions set forth) will be 95 capable of extensive use in the arts. Hence my process is not to be limited to the production of calcium carbide nor to the use of limestone as a fluxing agent.

Having thus described my invention what 95 I claim is:

1. The process of producing gas and carbide and reducing ore which comprises heating in a retort closed to the atmosphere a mixture of ore, limestone, and cokable carbonaceous material in proportions suitable to furnish the limestone and coke necessary for the carbide reaction and for the ore reduction, collecting the combustible gases evolved during the retorting operation, reducing the solid educt in an electric furnace thereby to obtain carbide and the metal of the ore, collecting the evolved combustible gases, and separating the metal and the carbide. 105

2. The process of producing carbide and reducing ore which comprises retorting a mixture of ore, limestone and cokable carbonaceous material in proportions suitable to furnish the limestone and coke necessary 115 for the carbide reaction and for the ore reduction and without material reduction of such limestone, and reducing the solid educt in an electric furnace thereby to produce carbide and the metal of the ore. 120

3. The process of producing a metallic carbide and reducing an ore which comprises retorting a mixture of such ore with cokable carbonaceous material and with a fluxing agent containing the metal ingredient of such carbide, collecting the evolved gases, reducing the solid educt in an electric furnace at a temperature sufficient to secure the carbide reaction, and collecting the evolved 125 gases. 130

4. The process of producing a metallic carbide and reducing an ore which comprises heating in a retort closed to the atmosphere a mixture of such ore with cokable carbonaceous material and with a carbonate containing the metal ingredient of such carbide, and reducing the solid educt in an electric furnace at a temperature sufficient to secure the carbide reaction.
5. Material for the production of carbide and reduction of ore consisting of a coked mixture of carbonaceous material with such ore and a fluxing agent containing the metal ingredient of the carbide.
- 10 6. Material for the production of carbide and reduction of ore consisting of a coked mixture of carbonaceous material with such ore and with limestone.
- 15 7. Material for the production of carbide

and reduction of iron ore consisting of coked mixture containing the following ingredients in about the proportions specified:

|           | Per cent. |
|-----------|-----------|
| Ore       | 27.7      |
| Coke      | 32.2      |
| Limestone | 40.1      |

8. Material for the production of carbide and reduction of iron ore consisting of a mixture containing the following ingredients in about the proportions specified:

|           | Per cent. |
|-----------|-----------|
| Ore       | 27.7      |
| Coke      | 32.2      |
| Limestone | 40.1      |

In testimony whereof, I hereunto affix my signature.

JAMES HENRY REID.